

## UNITED STATES PATENT OFFICE

2,158,147

## METHOD OF PRODUCING TEXTILE FABRICS

Herbert Platt, Cumberland, Md., assignor to Celanese Corporation of America, a corporation of Delaware

No Drawing. Application October 12, 1934, Serial No. 748,087. Renewed November 29, 1938

6 Claims. (Cl. 26—56)

This invention relates to the method of obtaining a desired width and to the stabilization of the width to washing, of such fabrics as knit and woven fabrics comprising yarns of an organic derivative of cellulose.

An object of the invention is to form a desired width fabric especially of the circular knit type economically and expeditiously.

Another object of the invention is the setting or stabilizing of the width of a fabric so that it is unaltered in washing, dyeing or any future contact with ordinary liquid baths or otherwise becoming wet. Other objects of the invention will appear from the following detailed description.

By this invention there may be made circular knit fabrics of any desired width with but a limited variety of sizes of circular knitting machines. Accordingly, it is not necessary to finish circular knit fabrics to a width slightly less than the greige width of the machine upon which they were knitted. This invention dispenses with the requirement of an endless number of machines of different diameter, especially machines with very large diameter and therefore very expensive, to make the different widths required in the trade for circular knit fabrics.

By this invention there is imparted to the fabrics the desired width and also the desirable property that the desired widths are permanent to washing, dyeing or other treatment and contact with aqueous baths normally met with in the processing of the fabric after its formation or those met with in use in respect to wearing apparel. This invention not only sets or makes permanent the width of a fabric but also sets or makes permanent the stitch shape or weave thereby reducing slipping, distortions and the grouping of yarns together which distortion and grouping of the yarns normally form thin and thick striation in the fabric.

By the employment of this invention a non-slipping fabric may be made of a fabric that normally allows slipping of weft over warp in woven fabrics or of stitches in knit material. Many novel effects may be produced by the change in shape of the weave or stitch from the normal to one altered, to any of a various number of shapes depending on the degrees of stretch imparted to the fabric, which change in shape is permanent and set. Thus, in the making of a voile, the weft and the warp will anchor each other so firmly that they form a non-slipping fabric.

This invention gives to the finisher a means of controlling and manipulating the circular knit fabrics, so that he can, within certain limits say

3 inches in a 20 inch fabric, place the circular knit fabric at the width or widths desired. All knit fabrics tend on wet treatment to assume a fixed length and width, depending on the build of the fabric, but this tendency can be controlled by the manipulation of the knit fabric according to this invention and the dyeing, drying and finishing processes, as well as treatments received in using the fabric, leave the width factor unaltered and as it was permanently set by the finisher.

According to my invention, I permanently stabilize or set to a desired or predetermined width a fabric, containing an organic derivative of cellulose, with or without other materials, by holding the fabric at said width while the fabric is in a wetted, softened or partially plastic state.

This invention is applicable to fabric formed by circular knitting, warp knitting, knotting, weaving or other fabrication of a textile fabric from yarns, threads, filaments, etc., a part of said yarns, etc. being formed of an organic derivative of cellulose. It is, however, especially applicable to circular knitted fabrics formed of a yarn consisting of an organic derivative of cellulose.

Accordingly, fabrics of the circular knit type may be stretched to the desired width and, while being held to said width, they may be wetted or made plastic by immersion for from 2 to 15 minutes in an aqueous bath containing from 5 to 20 grams per litre soap, said bath being maintained at about 98° C. After drying and/or cooling the fabric may be removed from the stretching device and subsequently dyed, calendered, washed and otherwise treated in the ordinary manner with but a negligible decrease in the width of the fabric. The width of the circular knit fabric may be set at the greige width, i. e. the width of the fabric as it comes from the loom or knitting machine or any width above the greige width, preferably not exceeding 4 inches of stretch in 20 inches for most of the ordinary cloths such as used in the underwear trade. For the purpose of producing novel effects, however, circular knit material may be formed with a more loose stitch than usual and the degree of stretch increased.

Accordingly, fabrics of the circular knit, warp knit or woven type may be treated by submerging same in an aqueous bath for 2 to 15 minutes, said bath being maintained at a temperature of about 98° C. and containing 5 to 20 grams per litre soap and the fabric then stretched to the desired width and held in a stretched condition until partially dried or cooled, after which it may be rewetted,

dyed, washed, calendered, etc. without an appreciable loss in width. Or the fabric, preferably of a circular knit type, may be treated with steam while wet with an aqueous bath containing 5 to 20 grams per litre soap by stretching the same to the desired width while applying the steam. Thus the wet circular knit fabric may be treated with steam while stretching it over a head, cone or cylinder having therein perforations 10 through which steam is emitted. Alternatively, any of the fabrics while wet may be passed through a steam bath or over a steam table while being held to the desired width by their marginal edges. The steam employed when using a cone, header or spreader may be either dry or wet steam and 15 may be under pressure, say about 5 lbs.

In dyeing fabrics formed of yarns containing organic derivatives of cellulose, there is often incorporated in the dye bath from 1 to 4 grams per 20 litre of soap and/or other compounds which are equivalent to soap for the purpose of placing the fabric in a wet or plastic condition. Thus the fabric may be stretched while in such a bath or it may be stretched in the presence of steam, before 25 drying, after removal from such a bath.

For the purpose of setting the width or for imparting a slight amount of stretch to a fabric, aqueous baths without soap may be employed and the wet fabric from such a bath may be given a 30 steam bath while being stretched preferably in the presence of wet steam. However, dry steam may be employed.

The yarns from which the textile fabric to be treated is formed may be composed of a single 35 filament, assemblies or bundles of a number of continuous filaments which may be in parallel relationship or which may be twisted together, straws, short lengths of staple fiber or threads or yarns spun from such staple fibers. This invention is particularly of importance in connection 40 with the fabrics made of yarns or filaments of organic esters of cellulose and organic ethers of cellulose. Examples of organic esters of cellulose are cellulose acetate, cellulose formate, cellulose propionate and cellulose butyrate, while examples of organic ethers of cellulose are ethyl cellulose, methyl cellulose and benzyl cellulose.

The yarns forming the textile fabric to be treated may be spun or drawn from an organic 50 derivative of cellulose solution by either the wet or dry method of spinning. They may contain effect materials such as pigments, filling materials such as the oxides of metals, dyes or lakes and/or effect materials such as fire retardants, sizes, plasticizers, softeners and lubricants. Examples of sizes are wax, gelatines and starches. Examples of the plasticizers and softeners are triethanolamine stearate and the glycol or glycerol stearates or oleates. Examples of the lubricants are the glycerides of fatty acids, oils, such as olive oil, etc. Any of the above or analogous 55 effect materials or mixtures of same may be added to the yarns or filaments by adding the same in suitable solvents or emulsifiers to the spinning solution from which the yarns or filaments or constituent fibers of the same are spun or drawn. Also they may be added to the yarns or filaments by treating the yarns or filaments with a swelling agent such as mono-ethyl ether of ethylene glycol and applying them to the swollen yarn or filament so that upon contraction of the yarn or filament they are imbedded therein.

The yarns or filaments of the textile fabric to be treated may contain in addition to the organic 75 derivative of cellulose and the above effect ma-

terials such other effect materials as threads, filaments or fibers of cotton, wool, silk, etc. These effect materials may be incorporated with the filaments, fibers, yarns, etc. of the organic derivative of cellulose by twisting them together while the organic derivative of cellulose is in a swollen or softened state. They may also be incorporated with filaments and straws by imbedding them in the straw or filament by softening the straw or filament and passing the effect material 10 and straw or filament through press rolls with or without heat.

This invention is also applicable to textiles or fabrics woven or knitted from two or more distinct types of yarns or filaments. Thus filaments 15 of an organic derivative of cellulose may be woven or knitted with yarns of cotton, wool, silk or other natural fiber or with regenerated cellulose. It is preferable, however, to employ this invention in connection with circular knit fabrics 20 formed for the most part of an organic derivative of cellulose.

For the purpose of further describing the invention but not with the intention of limiting it thereto, the following specific examples are given. 25

#### Example I

An olive oil treated yarn of twisted filaments containing cellulose acetate is circular knitted in usual manner such that its raw width is 24 $\frac{3}{4}$  30 inches. This is placed on a stretching frame increasing its width to 26 $\frac{1}{2}$  inches in which condition it is immersed in a bath containing 10 grams per litre soap for 15 minutes, said bath being maintained at 98° C. This fabric is dried while 35 stretched and when removed from the frame is found to maintain said width. This fabric is given a thorough washing and again dried and the width is found to measure 26 $\frac{1}{2}$ ''.

#### Example II

A circular knit fabric of yarns containing cellulose acetate made on a 26 inch machine after dyeing is treated while wet by passing it over a steam head and spreader thereby stretching it 45 to a width of 20 $\frac{1}{2}$ '' which fabric when dried, washed and dried measures 20 $\frac{3}{4}$ '' in width.

The foregoing detailed description and examples is merely given by way of illustration and many alterations may be made therein without departing from the spirit of my invention. 50

Having described my invention what I desire to secure by Letters Patent is:

1. Process for imparting a desired width to a knitted textile fabric containing filaments of an organic derivative of cellulose, which width is permanent to all subsequent wet treatment, which comprises stretching the said knitted textile fabric while the same is subjected to the action of a hot aqueous fluid at a temperature and for a duration of time sufficient to soften the organic derivative of cellulose filaments of said fabric.

2. Process for imparting a desired width to a knitted textile fabric containing filaments of cellulose acetate, which width is permanent to all subsequent wet treatment, which comprises stretching the said knitted textile fabric while the same is subjected to the action of a hot aqueous fluid at a temperature and for a duration of time sufficient to soften the cellulose acetate filaments of said fabric.

3. Process for imparting a desired width to a knitted textile fabric containing filaments of an organic derivative of cellulose, which width is 75

permanent to all subsequent wet treatment, which comprises stretching the said knitted textile fabric while the same is subjected to the action of a hot aqueous liquid at a temperature and 5 for a duration of time sufficient to soften the organic derivative of cellulose filaments of said fabric.

4. Process for imparting a desired width to a knitted textile fabric containing filaments of cellulose acetate, which width is permanent to all 10 subsequent wet treatment, which comprises stretching the said knitted textile fabric while the same is subjected to the action of wet steam for a duration of time sufficient to soften the cellulose acetate filaments of the fabric.

15 5. Process for imparting a desired width to a knitted textile fabric containing filaments of an organic derivative of cellulose, which width is

permanent to all subsequent wet treatment, which comprises maintaining said knitted textile fabric to the desired width while immersing the same in a hot aqueous bath containing soap, said bath causing the organic derivative of cellulose 5 filaments of the fabric to soften, and then drying said fabric.

6. Process for imparting a desired width to a knitted textile fabric containing filaments of cellulose acetate, which width is permanent to all 10 subsequent wet treatment, which comprises maintaining said knitted textile fabric to the desired width while immersing the same in a hot aqueous bath containing soap, said bath causing the cellulose acetate filaments of the fabric to 15 soften, and then drying said fabric.

HERBERT PLATT.